

## UNITED STATES PATENT OFFICE.

HAROLD F. WHITTAKER, OF CARNEYS POINT, NEW JERSEY, AND THEODORE BAKER, OF WILMINGTON, DELAWARE, ASSIGNORS TO E. I. DU PONT DE NEMOURS & COMPANY, OF WILMINGTON, DELAWARE, A CORPORATION OF DELAWARE.

## ENAMELED WARE.

No Drawing.

Application filed April 28, 1921. Serial No. 465,304.

To all whom it may concern:

Be it known that we, HAROLD F. WHITTAKER and THEODORE BAKER, citizens of the United States, and residents of Carneys Point, in the county of Salem and State of New Jersey, and Wilmington, in the county of New Castle and State of Delaware, respectively, have invented a certain new and useful Enamelled Ware, of which the following is a specification.

This invention relates to improvements in enameled ware in which an enamel of a glassy nature is fused onto a metallic base to produce apparatus of greater resistance to wear and corrosion than has the bare metal base.

In this industry the most commonly used metal bases are cast iron and steel; other metals are mostly less suitable either because of their prohibitive price, too great coefficient of expansion, or low melting point. The enamels for this work have to be most carefully chosen and compounded so that differences in expansion and contraction and their ill effects will be minimized, and this has been done to the detriment of the resistance of the enamel to corrosion, as will be explained in greater detail later on.

The object of our invention is to so compound the metal base by employing a suitable alloy that the expansion coefficient of the base is adjusted to suit that of the enamel, allowing the composition of this to be chosen as most suitable from every other point of view, especially that of chemical resistance.

As examples of the materials hitherto added to enamels to render their expansion and contraction similar to that of the iron or steel base there may be mentioned the oxides of iron, lead, cobalt and nickel, as well as certain compounds of boron and fluorine. These ingredients also materially lower the fusing point of the enamel and facilitate the burning on in a uniform layer. On the other hand, borax imparts to the enamel certain undesirable properties, among them being a solvent action on the opacifying agents and most important of all, it imparts to the enamel a decided susceptibility to corrosive action. The same is true, to some extent, of fluorides. Although fluor spar acts as an opacifier when added in large amounts, it is known to have, when present

to the extent of more than 3%, a decidedly 55 weakening effect upon the resistance of the enamel to the solvent action of acids, alkalies or water. The adjustment of the coefficient of expansion of the metal base will 60 make possible the use of a more acid resistant enamel, since the differential coefficient of expansion between the selected enamel and the metal base can be reduced to a very low figure and thus prevent the usual checking and chipping of the enamel 65 coating when subjected to temperature changes while in operation.

Our method of controlling the expansion coefficient of the iron or steel is to add, as an ingredient thereto, a suitable amount of 70 nickel with minor optional additions of such other materials as manganese, chromium, tungsten, vanadium, or cobalt.

The above method of adjusting or controlling the coefficient of expansion of the 75 metal base so that it will conform with that of the selected enamel, is illustrated by the following example. The iron or steel alloy, which is used as the base metal for the enamel coating, should have a composition 80 within the following limits.

|               | Per cent.    |    |
|---------------|--------------|----|
| Iron or steel | 50 to 68     |    |
| Nickel        | 32 to 43     | 85 |
| Chromium      | 0 to 10      |    |
| Carbon        | 0 to 0.2     |    |
| Manganese     | 0 to 1.0     |    |
| Phosphorus    | not over .05 |    |
| Sulphur       | not over .07 | 90 |

Due to the fact that the coefficients of expansion of the various enamels vary, it is evident that our invention is not limited to any one composition of corresponding base metal. The following examples of alloy 95 compositions which provide suitable metal bases for the above-described enamels having low coefficients of expansion are given to illustrate our invention in greater detail:—

|            | I.       | II.      | III.     | 100 |
|------------|----------|----------|----------|-----|
|            | Percent. | Percent. | Percent. |     |
| Iron       | 57.48    | 56.23    | 58.93    |     |
| Nickel     | 42.00    | 36.20    | 39.00    |     |
| Chromium   | .00      | 7.00     | 1.50     |     |
| Carbon     | .10      | .10      | .10      |     |
| Manganese  | .35      | .40      | .40      |     |
| Phosphorus | .03      | .03      | .03      |     |
| Sulphur    | .04      | .04      | .04      |     |

The manganese is added to improve the casting qualities of the alloy.

The presence of carbon in the iron or steel, even in amounts as small as .10 or 5 .20%, has a tendency, especially with certain proportions of iron and nickel, to cause wide fluctuations in the coefficient of expansion at different temperatures; this tendency is counteracted to a certain extent if chromium is present. The use of chromium is 10 also desirable for the reason that it facilitates an adjustment of the coefficient of expansion within certain limits. Thus for a nickel-iron alloy containing about 36% Ni 15 the coefficient of expansion varies, between  $2 \times 10^{-6}$  and  $7.5 \times 10^{-6}$ , almost directly as the percentage of chromium between 1 and 10%.

The composition of the enamel according 20 to our invention may approximate the composition of glasses in common use for laboratory ware, e. g.:-

|                            | Per cent. |
|----------------------------|-----------|
| 25 $\text{SiO}_2$          | 67        |
| $\text{B}_2\text{O}_3$     | 6.9       |
| $\text{Na}_2\text{O}$      | 8.5       |
| $\text{K}_2\text{O}$       | 0.4       |
| $\text{CaO}$               | 7.0       |
| $\text{MgO}$               | 0.2       |
| 30 $\text{Al}_2\text{O}_3$ | 10.0      |

The above enamel formula is, of course, merely illustrative; any enamel composition having high chemical resistance or other desirable properties incompatible with a high coefficient of expansion may be said to come 35 within the purview of our invention.

For example, many compositions of 40 enamels having the desired chemical and physical properties have components whose proportions come within the limits set forth in the following table:-

|                            | Per cent.    |
|----------------------------|--------------|
| 45 $\text{SiO}_2$          | 67.0 to 75.0 |
| $\text{B}_2\text{O}_3$     | 4.0 to 24.0  |
| $\text{Na}_2\text{O}$      | 4.0 to 8.5   |
| $\text{K}_2\text{O}$       | 0.2 to 1.3   |
| $\text{CaO}$               | 0.2 to 7.0   |
| $\text{MgO}$               | 0.0 to 0.5   |
| 50 $\text{Al}_2\text{O}_3$ | 0.0 to 10.0  |
| $\text{PbO}$               | 0.0 to 1.0   |

Although the invention has been described with particular reference to iron and steel, it will be understood that other metals or 55 alloys can be used. By the word "iron" in the claims we include both iron and steel.

We claim:-

1. In the method of making chemically 60 resistant enameled ware having a metallic base, the step which comprises incorporating in the base material a metal capable of rendering the coefficient of expansion of the metallic base substantially the same as the coefficient of expansion of the enamel component of said ware, shaping said base ma-

terial into the desired form, and applying thereto the enamel.

2. In the method of making chemically 70 resistant enameled iron, the step which comprises incorporating in the iron, before applying the enamel, sufficient nickel to form an alloy whose coefficient of expansion is substantially the same as that of the enamel component of said ware, shaping said base material into the desired form, and applying thereto the enamel. 75

3. As a new article of manufacture, enameled ware having a metallic base and comprising an enamel having high chemical 80 resistance and a relatively low coefficient of expansion, and a metallic base consisting of an alloy whose coefficient of expansion is substantially the same as that of the enamel.

4. As a new article of manufacture, an enameled iron alloy comprising an enamel having high chemical resistance and a relatively low coefficient of expansion, and a base consisting essentially of iron and a sufficient amount of another metal to form an alloy whose coefficient of expansion is substantially the same as that of the enamel. 90

5. As a new article of manufacture, an enameled iron alloy comprising an enamel having high chemical resistance and a relatively low coefficient of expansion, and a base consisting essentially of iron and a sufficient amount of nickel to form an alloy whose coefficient of expansion is substantially the same as that of the enamel. 95

6. As a new article of manufacture, an 100 enameled iron alloy comprising an enamel having a relatively low coefficient of expansion, and an alloy having substantially the same coefficient of expansion and containing between 50 and 68% of iron and between 105 43 and 32% of nickel.

7. As a new article of manufacture, an 110 enameled iron alloy comprising an enamel having a relatively low coefficient of expansion and high chemical resistance, and an alloy having substantially the same coefficient of expansion and consisting essentially of iron, nickel, and chromium.

8. As a new article of manufacture, an 115 enameled iron alloy comprising an enamel having a relatively low coefficient of expansion and high chemical resistance, and an alloy having substantially the same coefficient of expansion and containing between 50 and 68% of iron, between 43 and 32% of 120 nickel, and between 0.0 and 10% of chromium.

9. As a new article of manufacture, an 125 enameled iron alloy comprising an enamel having a relatively low coefficient of expansion and high chemical resistance, and an alloy having substantially the same coefficient of expansion and containing from about 58 to 60 parts of iron, about 39 parts of nickel, from about 1 to 2 parts of

chromium, about 0.1 part of carbon, and whose components are present in the following proportions:

10. As a new article of manufacture, an enameled iron alloy comprising an enamel whose components are present in the following proportions:

|    | Per cent.                      |
|----|--------------------------------|
| 10 | <chem>SiO2</chem> 67.0 to 75.0 |
|    | <chem>B2O3</chem> 4.0 to 24.0  |
|    | <chem>Na2O</chem> 4.0 to 8.5   |
|    | <chem>K2O</chem> 0.2 to 1.3    |
|    | <chem>CaO</chem> 0.2 to 7.0    |
|    | <chem>MgO</chem> 0.0 to 0.5    |
| 15 | <chem>Al2O3</chem> 0.0 to 10.0 |
|    | <chem>PbO</chem> 0.0 to 1.0    |

and an alloy having substantially the same coefficient of expansion as said enamel.

11. As a new article of manufacture, an enameled iron alloy comprising an enamel

|  | Per cent.                      |    |
|--|--------------------------------|----|
|  | <chem>SiO2</chem> 67.0 to 75.0 | 25 |
|  | <chem>B2O3</chem> 4.0 to 24.0  |    |
|  | <chem>Na2O</chem> 4.0 to 8.5   |    |
|  | <chem>K2O</chem> 0.2 to 1.3    |    |
|  | <chem>CaO</chem> 0.2 to 7.0    |    |
|  | <chem>MgO</chem> 0.0 to 0.5    |    |
|  | <chem>Al2O3</chem> 0.0 to 10.0 | 30 |
|  | <chem>PbO</chem> 0.0 to 1.0    |    |

and an alloy having substantially the same coefficient of expansion as said enamel and containing between 50 and 68% of iron and between 43 and 32% of nickel.

In testimony whereof we affix our signatures.

HAROLD F. WHITTAKER.  
THEODORE BAKER.